

No. 730,155.

PATENTED JUNE 2, 1903.

G. PY.

TREATMENT OF PEAT FIBER.

APPLICATION FILED JULY 30, 1900.

NO MODEL.



Witnesses

  


Inventor

George Py  
by James L. Morris.  
atty

## UNITED STATES PATENT OFFICE.

GEORGES PY, OF PARIS, FRANCE.

## TREATMENT OF PEAT FIBER.

SPECIFICATION forming part of Letters Patent No. 730,155, dated June 2, 1903.

Application filed July 30, 1900. Serial No. 25,326. (No specimens.)

*To all whom it may concern:*

Be it known that I, GEORGES PY, chemist, a citizen of the Republic of France, residing at 68 Rue du Landy, Plaine St. Denis, Paris, France, have invented certain new and useful Improvements in the Treatment of Peat Fiber, of which the following is a specification.

This invention relates to the treatment of peat fiber, and has for its chief object the rapid and economical conversion of peat fiber into fleece for use either alone or with any other textile material, a larger proportion of fleece being obtained from the quantity of peat used than has hitherto been accomplished.

Hitherto the processes employed for the treatment of peat have only concerned the separation and utilization of vegetable fiber already isolated by the partial fermentation to which plants are subjected during the formation of peat. This separation, effected by successive cardings, has the great commercial objection that a small yield of useful fiber and a large amount of waste material are obtained, this objection being greater when the manufacture of the fiber takes place at some distance from the locality where the peat is obtained.

Now the present process is a retting process, in which the complete extraction of all useful separable or ligneous fibers is obtained by a chemical process and remarkable absorbent properties are imparted to such fibrous material, while also rendering the said material suitable for carding, combing, spinning, or weaving. The fleece produced by this process of treatment does not require special machines for working it and can be used either alone or in combination or conjunction with other textile materials of manufacture.

According to the present invention the fibrous material after it has been beaten to free it from earthy matter and the stalks, roots, and foreign substances have been removed is first subjected to the action of an alkaline solution. After being removed from this solution and washed the said fibrous material is treated under pressure with a weak solution of sulfuric acid. It is then allowed to drain and after being heated in a strong solution. The fibrous material is rendered neutral by means of an alkali and softened by soapy water.

In order that the invention may be clearly understood and readily carried into effect, the same will now be described more fully with reference to the accompanying drawing. It is to be understood that this drawing is by way of example only, illustrating means whereby the process may be carried into practice.

The fibrous material freed from dirt and earthy matter is introduced into a double cylinder A, preferably constructed of enameled-iron plates. The inner cylinder a is perforated and is rotated in either direction around its axis a' by suitable gearing, while the external cylinder b is stationary and constructed in such a manner as to be capable of supporting a pressure of about four kilograms per square centimeter. The said cylinder is supplied with water, steam, and the requisite chemicals through pipes c d e, respectively. A sufficient quantity of water rendered alkaline by the addition of potash, lime, soda, or ammonia is admitted to the cylinder in sufficient quantity to submerge the fibrous material therein. The weight of the alkali used in the bath is preferably two per cent. of the weight of the fibrous material under treatment. When the action of this alkaline solution has reached the necessary limit, it is run off, and the fibrous material is rinsed or washed once or twice with water and afterward subjected to the action, under pressure, of from two to three per cent. solution of sulfuric acid. The duration of this operation may vary from one-half hour to two hours, according to the height of the pressure or to the strength of the acid-bath. The fibrous material is afterward removed from the cylinder, allowed to drain, and then subjected to the action of a strong solution of oxalic, hydrochloric, or sulfuric acid. The concentration of the said acids may vary from 45° Baumé to 19° Baumé, according to whether the troughs are furnished with lead serpentine tubes permitting an elevation of 95 temperature. The action of the acids under heat requires watching very carefully, because a maximum concentration, for example, of 45° coinciding with an elevation by one degree might cause the alteration and even the destruction of the fibrous material. After removing the fibrous material from the acid-bath it is introduced into a washing apparatus, which may consist of what is known as a

6c

70

75

80

85

90

95

100

"fulling-trough," "rinsing-barrel," or other apparatus, in which the said material is neutralized by the addition of an alkali and then rendered supple by means of soapy water. 5 This last operation of washing must produce a slight felting action of the fibrous material. The fibrous material thus purified is now isolated and clean and free from the excess of earthy derivatives and resinous matters with- 10 out, however, losing its most essential property—viz., that of resisting microbial fermentation. For its conversion into fleece the fibrous material is subjected, first, to a beating operation and then to a carding action in 15 an appropriate carding-machine, which may or may not be furnished with movable cards designed to sustain and give a greater cohesion to the nap. According to the fineness desired to be given, a teasing-cylinder with a venti- 20 lator may or may not be employed.

When the fleece is intended for surgical purposes, the fibrous material is subjected to a special combing operation in any convenient apparatus for freeing it of all dust and 25 woody matter that have remained. This fleece is made up into packets wrapped in impermeable bacteriological paper and is sterilized at 134° centigrade under pressure, and if not required for immediate use is wrapped in 30 paraffin-paper and sealed either with paraffin, wax, or any suitable adhesive resinous substance which is soluble in alcohol.

If it is desired to completely bleach the peat fiber, I agitate it in a five-per-cent. soda solution under a pressure of two to four kilos per 35 square centimeter until the whole of the earthy derivatives soluble in alkalies have been removed, after which the bleaching operation may be completed by any of the usual 40 processes.

What I claim is—

1. A process for the treatment of peat fiber to obtain a fleece, consisting in subjecting

the said fiber to the action of an alkali solution, washing it and treating it under pressure with a weak solution of acid, then draining it and heating it with a strong solution of acid, then washing and neutralizing it, said alkali and acid solutions all having a temperature and degree of concentration insufficient 45 to convert the fiber into a pulp. 5c

2. A process for the treatment of peat fiber to obtain a fleece, consisting in subjecting the said fiber to the action of a solution containing about two per cent. of the weight of 55 the fiber of alkali, washing said fiber, subjecting said fiber for from one-half hour to two hours to the action of a solution containing from two per cent. to three per cent. of acid, draining said fiber, and subjecting said fiber 6c to the action of a solution at from 19° to 45° Baumé of acid at a temperature to sufficiently accelerate the action of said acid, but not sufficient to pulp the fiber, substantially as described. 65

3. A process for the preparation of a fleece suitable for surgical purposes, consisting in subjecting mechanically-cleaned peat fiber to the action of an alkali solution, washing it and treating it under pressure with a weak 70 solution of acid, then draining it and heating it with a strong solution of acid, then washing and neutralizing it, and afterward softening and felting it by means of soapy water, the aforesaid alkali and acid solutions all 75 having a temperature and degree of concentration insufficient to convert the fiber into a pulp, substantially as described.

In testimony whereof I have hereunto set my hand, in presence of two subscribing witnesses, this 19th day of July, 1900.

GEORGES PY.

Witnesses:

HENRI CLAUZIER,  
EDWARD P. MACLEAN.